

# UNITED STATES PATENT OFFICE.

HAROLD EDWIN CLEAVES, OF WASHINGTON, DISTRICT OF COLUMBIA.

## PROCESS OF TREATING ALLOYS.

1,235,655.

Specification of Letters Patent.

Patented Aug. 7, 1917.

No Drawing.

Application filed May 23, 1917. Serial No. 170,522.

To all whom it may concern:

Be it known that I, HAROLD EDWIN CLEAVES, a citizen of the United States, residing at Washington, in the District of Columbia, have invented new and useful Improvements in Processes of Treating Alloys, of which the following is a specification.

This invention relates to a process of separating from each other metals which are intimately associated in their metallic state; and it comprises subjecting such a metal mixture to the action of a hydrogen halid, such as hydrogen chlorid, while maintaining the mixture at a temperature, usually above a red heat, at which at least one of the metals will be converted into a metal halid and volatilized.

The alloys and metal compositions with which the present process is chiefly concerned are those containing on the one hand a metal which is comparatively chemically inactive in the metallic state, such as the metals of the fifth and sixth groups of the periodic system, and particularly the metals: vanadium, chromium, molybdenum, and tungsten; and on the other hand, a metal such as iron which is comparatively active, and which will combine readily with hydrogen chlorid to form a metal chlorid.

The ferro-alloys such as ferrochromium, ferrotungsten, etc., obtainable, for instance, by reduction of their corresponding oxygen salts (chromites, tungstates) can be treated with great advantage by this process, the resulting products having a very low iron content, as well as a decreased percentage of sulfur, arsenic and oxygen if these metalloids were present in the original alloy.

The manner in which my process is carried out may be illustrated by the following examples:

Example I: A ferrotungsten, finely subdivided, containing about 70% tungsten, 25% iron, 1-2%  $WO_3$ , and small proportions of sulfur and manganese, is maintained at a temperature of about 1100° C and a stream of hydrogen chlorid gas passed over the heated material. The iron in the alloy is rapidly converted into iron chlorid, volatilized and removed by the stream of gas, the impurities oxygen, manganese, and sulfur being removed at the same time. The resulting product is almost pure metallic tungsten. The tungsten which was present as tungsten oxid is converted into tungsten chlorid and volatilized, but may be easily re-

covered from the gas mixture by suitable methods of condensation.

Example II: Ferromolybdenum, containing 60 to 70% molybdenum, is subjected in a finely subdivided condition to the action of hydrogen chlorid while maintained at a temperature of from 1050 to 1100° C. The iron is volatilized as iron chlorid and any molybdenum which was present as oxid is also volatilized in its chlorid form. The reaction is discontinued when the molybdenum content of the ferromolybdenum has been raised to about 90%, which can be accomplished in a comparatively short time.

Example III: Finely divided ferrochrome containing about 60% chromium is maintained at a temperature of about 1050° C. while hydrogen chlorid is passed in contact therewith. In this case both the chromium and iron are converted into their chlorids, but only the iron chlorid is volatilized. A very effective separation of the iron and chromium is thereby obtained, the chromium being in a form readily convertible into other valuable chromium compounds.

Example IV: Ferrovanadium, suitably comminuted, and containing about 70% vanadium, is maintained at a temperature of about 1050° C. while a stream of hydrogen chlorid is passed in contact therewith. The iron is volatilized as the chlorid, leaving metallic vanadium from which most, if not all, of the iron has been removed. Any impurities such as oxygen and sulfur are removed at the same time.

My invention includes a fractional, as well as a complete, removal of one of the components of the metal mixture or alloy, since in many cases the presence of one of the components, such as iron, in small proportions is not objectionable.

What I claim is:

1. The process of treating a metal mixture or alloy to reduce the content of one of the component metals, at least one of the component metals being capable of reacting with hydrogen halid to form a metal halid volatile at a high temperature, which comprises subjecting the suitably subdivided metal mixture to the action of hydrogen halid while maintaining said mixture at a temperature at which the halid of at least one of the metals is formed and volatilized.

2. The process of treating a metal mixture or alloy to reduce the content of one of the component metals, at least one of the

- component metals being capable of reacting with hydrogen chlorid to form a metal chlorid volatile at a high temperature, which comprises subjecting the suitably subdivided metal mixture to the action of hydrogen chlorid while maintaining said mixture at a temperature at which the chlorid of at least one of the metals is formed and volatilized.
5. The process of reducing the iron content of a ferro-alloy of vanadium, tungsten or molybdenum, which comprises passing hydrogen chlorid in contact with said alloy while maintaining the latter at a temperature of about from 1000 to 1100° C.
10. 3. The process of treating metals of the fifth and sixth groups of the periodic system intimately associated with a metal capable of reacting with hydrogen chlorid to form a metal chlorid, which comprises passing hydrogen chlorid in contact with the finely divided metal mixture, while maintaining the latter at a temperature at which said metal chlorid will be formed and volatilized.
15. 4. The process of reducing the iron content of a ferro-alloy of vanadium, tungsten or molybdenum, which comprises passing hydrogen chlorid in contact with said alloy while maintaining the latter at a tempera-
- ture at which iron chlorid will be formed and volatilized.
5. The process of reducing the iron content of a ferro-alloy of vanadium, tungsten or molybdenum, which comprises passing hydrogen chlorid in contact with said alloy while maintaining the latter at a temperature of about from 1000 to 1100° C.
6. The process of reducing the iron content of a ferrotungsten which comprises passing hydrogen chlorid in contact with finely divided ferrotungsten while maintaining the latter at a temperature at which iron chlorid will be formed and volatilized.
7. The process of removing iron from a ferrotungsten containing more tungsten than iron, which comprises subjecting said ferrotungsten, in a suitably finely divided condition, to the action of hydrogen chlorid while maintaining the ferrotungsten at a temperature of about 1000 to 1100° C.
- In testimony whereof I affix my signature.

HAROLD EDWIN CLEAVES.